

## UNITED STATES PATENT OFFICE.

LESLIE G. JENNESS, OF LEONIA, NEW JERSEY.

## DRY-CELL ELEMENT AND METHOD OF MAKING THE SAME.

No Drawing.

Application filed February 18, 1927. Serial No. 169,419.

This invention relates to improvements in the method of preparing bobbins for use in dry cells, and more particularly for the galvanic cells of the bag type. In this type of cell, the active elements consist of a carbon rod, surrounded by a mixture of manganese dioxide and finely ground carbon or graphite, an electrolyte of ammonium chloride and zinc chloride, and a zinc cup. The manganese dioxide and carbon are molded around the carbon rod and this, commonly termed the bobbin, is usually wrapped in gauze, cheese cloth, or like fabric, before insertion into the zinc cup containing the electrolyte. The purpose of this cloth is to prevent the bobbin from becoming disintegrated during the process of insertion and the preparation of the cell, thereby causing a short circuit within the cell.

The step of wrapping these bobbins is expensive, both because of the cost of cloth and also because of the cost of the labor of applying the cloth. Heretofore, attempts have been made to avoid the necessity of wrapping the cells with cloth by making an insoluble coating or envelope upon the surface of the bobbins. These methods involved some process, such as dipping in one or more solutions, to replace that of wrapping with cloth. By the present invention, I eliminate this wrapping process without the substitution of any other process and without replacing the cloth with an insoluble coating or envelope upon the surface of the bobbins.

I have found that when an alkali metal salt, such as calcium chloride, for example, and a sulphate or a carbonate are added in the dry state to the bobbin mix before molding, that after molding, these bobbins will be sufficiently hard to have sufficient mechanical strength to allow the handling that is necessary to complete the process of assembling the battery. Although different sulphates may be used, I have found aluminium sulphate to be preferable. The chemical reaction which takes place between these substances, added in this manner, is slow and allows a good workability of the mix during the process of molding the bobbins. After a period of two days, the bobbins are sufficiently hard and strong to allow their insertion into the cups without wrapping in cloth and without danger of disintegration. It has been found that after

the completion of the battery, these bobbins remain in a hard condition for nearly a day. After the bobbins have been in contact with the electrolyte for a period greater than one day, they begin to soften to such an extent that the internal resistance of the battery is even less than that of batteries that have been wrapped in a cloth and made up without the addition of these substances. At this stage, however, there is no danger of disintegration of the bobbins since they are held in place by the pasty condition of the electrolyte. The materials mentioned above may be used in varying amounts, but I prefer to use about one per cent of aluminium sulphate (alum may also be used satisfactorily) and one half of one per cent of calcium chloride, and prefer to have an excess of aluminium sulphate present. These materials are not injurious to the battery. On the contrary, it has been found that batteries produced in this manner have a voltage in excess of batteries made in the usual manner, and that the "shelf life" is considerably increased.

During the interaction of the above mentioned substances, calcium sulphate is produced and the hardening properties of the molded bobbin are largely due to the formation of this compound. Calcium sulphate, when freshly precipitated, is somewhat soluble in water and much more soluble in mineral acids, such as hydrochloric acid. It is well known that zinc chloride, upon hydrolysis in aqueous solutions, yields hydrochloric acid and, therefore, this acid is always present in the electrolyte of the cell. For this reason, and the fact that an excess of aluminium sulphate is present which is soluble in water, the bobbins become soft after coming in contact with the electrolyte, due to the dissolving of the substances which have previously caused the hardness.

This invention is not limited to the formation of calcium sulphate in the bobbin, as other compounds, such as barium or other carbonates or certain salts of silicic acid which have the property of hardening soon after being formed and becoming soft by contact with hydrochloric acid, will produce similar results. I have found that, for example, calcium carbonate will, when produced within the bobbin, cause hardening of the bobbins and will, in turn, soften when in contact with

the electrolyte. Furthermore, aluminium sulphate alone will cause a slight hardening of the bobbins.

I claim:

5. 1. The method of producing bobbins which comprises adding substances, which will cause precipitation of a substance that will give hardness to the bobbin, to the bobbin ingredients and molding said substances with the bobbin ingredients.
10. 2. The method of producing bobbins which comprises adding substances, one of which is a sulphate, which will cause precipitation of a substance that will give hardness to the bobbin, to the bobbin ingredients and molding said substances with the bobbin ingredients.
15. 3. The method of producing bobbins which comprises adding substances, one of which is an alkali metal salt, which will cause precipitation of a substance that will give hardness to the bobbin, to the bobbin ingredients and molding said substances with the bobbin ingredients.
20. 4. The method of producing bobbins which comprises adding a soluble alkaline earth metal salt and a soluble sulphate to the bobbin ingredients and molding said substances with the bobbin ingredients.
25. 5. The method of producing bobbins which comprises adding a calcium salt and a soluble sulphate to the bobbin ingredients and molding said substances with the bobbin ingredients.
30. 6. The method of producing bobbins which comprises adding a calcium chloride and a soluble sulphate to the bobbin ingredients and molding said substances with the bobbin ingredients.
35. 7. The method of producing bobbins which comprises adding a calcium chloride and an aluminium salt to the bobbin ingredients and

molding said substances with the bobbin ingredients, said aluminium salt being one that will produce a hardening compound by reacting with calcium chloride.

45

8. The method of producing bobbins which comprises adding about one half of one percent of calcium chloride and about one percent of an aluminium salt to the bobbin ingredients and molding said substances with the bobbin ingredients, said aluminium salt being one that will produce a hardening compound by reacting with calcium chloride.

50

9. A battery bobbin comprising manganese dioxide and carbon mixed with ingredients that will react upon each other to harden the mixture in about two days and form a compound that is soluble in dilute hydrochloric acid.

55

10. A battery bobbin comprising manganese dioxide and carbon mixed with the reaction products of calcium chloride and aluminium sulphate.

60

11. A battery bobbin comprising manganese dioxide and carbon mixed with the reaction products of about one half of one percent of calcium chloride and one percent of aluminium sulphate.

65

12. The method of producing bobbins which comprises adding a calcium chloride and aluminium sulphate to the bobbin ingredients and molding said substances with the bobbin ingredients.

70

13. A battery bobbin comprising manganese dioxide and carbon mixed with a water-insoluble hardening salt substantially uniformly distributed in the depolarizing mix.

75

14. A battery bobbin comprising manganese dioxide and carbon mixed with calcium sulphate.

LESLIE G. JENNESS.